

# United States Patent [19]

Mihayashi et al.

[11] Patent Number: 4,656,123

[45] Date of Patent: Apr. 7, 1987

[54] SILVER HALIDE LIGHT-SENSITIVE MATERIAL COMPRISING A FOGGANT-RELEASING COUPLER AND A NON-DEVELOPABLE SILVER HALIDE LAYER BETWEEN COLOR-SENSITIVE EMULSION LAYERS

[75] Inventors: Keiji Mihayashi; Hidetoshi Kobayashi, both of Kanagawa, Japan

[73] Assignee: Fuji Photo Film Co., Ltd., Kanagawa, Japan

[21] Appl. No.: 695,132

[22] Filed: Jan. 25, 1985

## [30] Foreign Application Priority Data

Jan. 25, 1984 [JP] Japan 59-11745

[51] Int. Cl.<sup>4</sup> G03C 1/46; G03C 1/00; G03C 1/08; G03C 7/32

[52] U.S. Cl. 430/543; 430/505; 430/598; 430/955

[58] Field of Search 430/598, 955, 505, 543

## [56] References Cited

### U.S. PATENT DOCUMENTS

4,358,528 11/1982 Takagi et al. 430/598  
4,518,682 5/1985 Kobayashi et al. 430/543

4,526,863 7/1985 Mihayashi et al. 430/543

### FOREIGN PATENT DOCUMENTS

0117511 9/1984 European Pat. Off. 430/598  
0127081 12/1984 European Pat. Off. 430/598  
2131188 6/1984 United Kingdom .

Primary Examiner—John E. Kittle

Assistant Examiner—Mukund J. Shah

Attorney, Agent, or Firm—Sughrue, Mion, Zinn, Macpeak and Seas

## [57] ABSTRACT

A silver halide light-sensitive material is described, comprising a support having provided thereon at least two silver halide emulsion layers differing in color sensitivity, wherein at least one of said layers contains at least one compound capable of releasing a fogging agent, a development accelerator, or a precursor thereof in proportion to the amount of silver developed, and a layer containing silver halide grains which are not substantially developed by the development processing of said material is provided between said two emulsion layers differing in color sensitivity. The material has improved color reproducibility.

19 Claims, 1 Drawing Figure





**SILVER HALIDE LIGHT-SENSITIVE MATERIAL  
COMPRISING A FOGGANT-RELEASING  
COUPLER AND A NON-DEVELOPABLE SILVER  
HALIDE LAYER BETWEEN COLOR-SENSITIVE  
EMULSION LAYERS**

**FIELD OF THE INVENTION**

This invention relates to a silver halide light-sensitive material containing a compound capable of imagewise releasing a fogging agent or a development accelerator or a precursor thereof to thereby increase sensitivity and contrast or to accelerate development. More particularly, this invention relates to a silver halide color photographic light-sensitive material having improved color reproducibility.

**BACKGROUND OF THE INVENTION**

With recent developments in silver halide photographic light-sensitive materials, particularly light-sensitive materials for photography, light-sensitive materials having high sensitivity, as typically exemplified by films of ISO 1000, have become strongly desired. Various methods to increase sensitivity have hitherto been attempted by, for example, increasing the size of the silver halide grains increasing activity of couplers, accelerating development, and the like. However, any further increase in sensitivity by using large-sized silver halide grains cannot be expected, seeing that achievement in increasing sensitivity by using large-sized silver halide grains seems to have reached the limitation as reported in G. C. Farnell and J. B. Chanter, *Journal of Photographic Science*, Vol. 9, 75 (1961). Furthermore, increasing the grain size is accompanied with various disadvantages, such as deterioration in improved graininess or preservability of an emulsion layer in projection to increasing thickness. Further, use of highly active couplers or acceleration of development is not only accompanied by significant deterioration in graininess, but such is also insufficient in contributing to increases in sensitivity. Furthermore, addition of various development accelerators, such as hydrazine compounds, to an emulsion layer or a developing solution, typically in achromatic light-sensitive materials, has been studied for the purpose of accelerating development. However, conventional development accelerators are not fully satisfactory due to a tendency to increase fog and/or deteriorate graininess.

Hence, couplers capable of imagewise releasing a development accelerator or a fogging agent have been proposed. For example, U.S. Pat. Nos. 3,214,377 and 3,253,924 and Japanese Patent Application (OPI) No. 17437/76 (the term "OPI" as used herein means an "unexamined published application") disclose couplers capable of releasing thiocyanate ions which accelerate a physical phenomenon of dissolution. Further, Japanese Patent Application (OPI) No. 138636/82 discloses couplers capable of releasing hydroquinone or aminophenol developing agents.

However, the groups released from these couplers exhibit insufficient development accelerating activity or fogging activity so that use of these couplers brings about only a little effect. In order to overcome this problem, couplers capable of releasing acylhydrazines as described in Japanese Patent Application (OPI) No. 150845/72 and couplers capable of releasing thiocarbonyl compounds as described in Japanese Patent Appli-

cation (OPI) No. 161515/82 have been proposed to realize increase of sensitivity of means of couplers.

Nevertheless, since the released groups from these couplers are highly diffusible, when the couplers are incorporated in a layer sensitive to a certain color, the released compound is also diffused into other layers sensitive to a different color to thereby exhibit development accelerating activity or fogging activity therein, thus causing color mixing. Therefore, use of these couplers turns out to be disadvantageous in that color reproducibility is extremely deteriorated.

More specifically, in light-sensitive materials containing a compound capable of imagewise releasing of a fogging agent or a development accelerator or a precursor thereof (hereinafter referred to as "FR compound", and the compound capable of releasing FR compounds is hereinafter referred to as "FR-releasing compound") in accordance with the amount of developed silver, the FR compound released upon development donates an electron to the silver halide in the light-sensitive material or forms silver sulfide to increase centers of development, and thus accelerates development. As a result, favorable effects, such as an increase in sensitivity, increase in contrast, acceleration of development, and the like can be attained. On the other hand, a part of the FR compound imagewise released in a layer having a certain color sensitivity diffuses into other layers having different color sensitivity and accelerates development imagewise of said color sensitivity over unnecessarily enlarged portions of the light-sensitive material. This results in significant color mixing and extreme deterioration of color reproducibility.

Various other additives have also been studied in to increase sensitivity, but did not succeed due to considerable side effects.

**SUMMARY OF THE INVENTION**

One object of this invention is to provide a silver halide photographic light-sensitive material having high sensitivity and excellent color reproducibility.

Another object of this invention is to provide a silver halide photographic light-sensitive material which is excellent in rate of development and color reproducibility.

A further object of this invention is to provide a silver halide photographic light-sensitive material which exhibits improved color reproducibility while containing a reduced amount of silver.

As a result of extensive investigations to prevent diffusion of an FR compound from a particular color-sensitive emulsion layer in which the FR compound would be expected to act in other emulsion layers having a different color sensitivity, the present invention has finally been accomplished.

Thus, the objects of this invention can be accomplished by a silver halide photographic light-sensitive material comprising a support having provided thereon at least two emulsion layers differing in color sensitivity, at least one of said emulsion layers containing at least one compound capable of releasing a fogging agent, a development accelerator, or a precursor thereof in proportion to the amount of silver developed, upon development, wherein a layer containing silver halide grains which are not substantially developed by development processing of the light-sensitive material is provided between the two emulsion layers differing in color sensitivity.

That is, an important feature of the present invention involves providing a layer containing silver halide grains which are not substantially developed even after deactivation of an FR compound (hereinafter referred to "non-developable silver halide") between a color-sensitive emulsion layer containing an FR compound and a layer having a different color sensitivity. In order to deactivate an FR compound, it is preferable to use silver halide grains having a large surface area so as to have increased frequency of reaction, i.e., by using fine silver halide grains, and also to use a silver halide emulsion which is not developed by an ordinary surface developing solution even if an electron is donated by the FR compound to be deactivated, e.g., an emulsion having low sensitivity especially an internal latent image type silver halide emulsion.

Thus, fine silver halide grains as hereinafter described are effective to deactivate an FR compound, and the objects of the present invention can be achieved by providing a layer containing such silver halide grains between two silver halide emulsion layers differing in color sensitivity to different colors in a light-sensitive layer containing an FR-releasing compound, preferably in such a manner that said layer directly contacts with the two emulsion layers differing in color sensitivity.

#### BRIEF DESCRIPTION OF THE DRAWING

FIG. 1 is a graph showing interlayer effect from a red-sensitive emulsion layer to a green-sensitive emulsion layer or a degree of color mixing.

#### DETAILED DESCRIPTION OF THE INVENTION

FR-releasing compounds which can effectively be used in the present invention include compounds capable of releasing at least one of fogging agents, silver sulfide-forming agents, and silver halide solvents. These compounds release FR compounds upon reacting with an oxidation product of a developing agent which is formed when silver halides are reduced to silver by development processing.

FR compounds which can be used in the present invention include the following examples (i) to (iii). The symbol "FA" as used herein indicates a fogging agent, a development accelerator or precursors thereof.

- (i) Couplers capable of releasing FA upon coupling with an oxidation product of an aromatic primary amine developing agent.
- (ii) Couplers capable of forming a diffusible coupling product which functions as FA upon coupling with an oxidation product of an aromatic primary amine developing agent.
- (iii) Redox compounds capable of releasing FA upon oxidation-reduction reaction with an oxidation product of an aromatic primary amine developing agent or the subsequent reaction.

These compounds (i), (ii) and (iii) can be represented by the following formulae (1), (2) and (3), respectively.



wherein Cp represents a coupler residue capable of coupling with an oxidation product of an aromatic primary amine developing agent; BALL represents a non-

diffusible group which is eliminated from Cp upon the coupling reaction with an oxidation product of an aromatic primary amine developing agent; RED represents a residue of a compound capable of undergoing oxidation-reduction reaction with an oxidation product of an aromatic primary amine developing agent; TIME represents a timing group releasable from Cp or RED upon coupling reaction or oxidation-reduction reaction to release FA; n represents 0 or 1; FA represents a group releasable from Cp or RED upon coupling when n is 0, or a group releasable from TIME when n is 1.

In the above-described formula (2), FA may not be released from Cp or TIME after the coupling reaction.

In the above-described formulae (1), (2) and (3), FA represents a so-called fogging agent which reacts with silver halide grains during development to form a fog nucleus capable of starting development. FA includes groups which reductively react with silver halide grains to form fog nuclei and groups which react with silver halide grains to form silver sulfide nuclei capable of starting development.

Preferred FA groups are those containing a group having an adsorbing property onto silver halide grains and can be represented by the formula:



wherein AD represents a group adsorptive onto silver halide grains; L represents a divalent group; m represents 0 or 1; and X represents a reducing group or a group capable of reacting with silver halide to form silver sulfide; with proviso that when X is a group capable of reacting with silver halide to form silver sulfide and also has a function of AD, the group  $AD-(L)_m-$  is not necessarily required.

When FA is a group represented by  $AD-(L)_m-X$ , it may be bonded to TIME, Cp or RED at an optional position of  $AD-(L)_m-X$ .

In the formula (1),  $-(TIME)_n-FA$  is bonded to the coupling position of Cp, and the bond is cleaved upon coupling reaction.

In the formula (2),  $BALL$  is bonded to Cp at the coupling position thereof, and the bond is cleaved upon coupling reaction. Since  $-(TIME)_n-FA$  is bonded to Cp at the non-coupling position thereof, this bond is not cleaved directly by the coupling reaction.

In the formula (3),  $-(TIME)_n-FA$  is bonded to RED at such a position that  $-(TIME)_n-FA$  is released therefrom by the oxidation-reduction reaction with an oxidation product of an aromatic primary amine development agent or the subsequent reaction.

The group represented by TIME may be trivalent group in the formula (1). Such being the case, one of the three bonds is bonded to FA and one of the remaining two bonds is bonded to the coupling position of Cp, with the other being bonded to the non-coupling position of Cp. When a compound having such a bond-structure is reacted with an oxidation product of an aromatic primary amine developing agent, the bond between TIME and the coupling position of Cp is cleaved, but the bond at the non-coupling position is not split off. The bond between TIME and FA is then cleaved through electron transfer reaction and/or intramolecular nucleophilic substitution of the anion, i.e., cleaved bond, of TIME whereby FA is released. Therefore, such a compound having a trivalent TIME should also have a structure capable of releasing FA by intra-

molecular electron transfer reaction and/or intramolecular nucleophilic substitution reaction.

The FR compounds represented by the aforesaid formulae (1), (2) and (3) will further be described in detail below.

In the formula (1), the coupler residue as represented by Cp has a partial structure of yellow, magenta and cyan couplers as well as colorless couplers and black-forming couplers.

Typical examples of the yellow couplers are described in U.S. Pat. Nos. 2,875,057, 2,407,210, 3,265,506, 2,298,443, 3,048,194 and 3,447,928, etc. Of these yellow couplers, acylacetamide derivatives, such as benzoylacetanilide, pivaloylacetanilide, etc., are preferred.

Accordingly, yellow coupler residues as Cp preferably include those represented by the formulae (I) and (II):



(I)

20



(II)

25

wherein the asterisk (\*) indicates a position to which FA or TIME is bonded (hereinafter the same up to formula (XV)); R<sub>1</sub> represents a nondiffusible group having from 8 to 32 total carbon atoms; and R<sub>2</sub>, which may be the same or different when R<sub>2</sub> represents 2 or more groups, represents a hydrogen atom or one or more of a halogen atom, a lower alkyl group, a lower alkoxy group and a nondiffusible group having from 8 to 32 total carbon atoms.

Typical examples of the magenta couplers are described in, e.g., U.S. Pat. Nos. 2,600,788, 2,369,489, 2,343,703, 2,311,082, 3,152,896, 3,519,429, 3,062,653 and 2,908,573, Japanese Patent Publication No. 27411/72 and Japanese Patent Application (OPI) Nos. 171956/84 and 162548/84, etc. Of these, pyrazolones and pyrazoloazoles (e.g., pyrazolopyrazole, pyrazoloimidazole, pyrazolobenzimidazole, pyrazolotriazole, pyrazolotetrazole, etc.) are preferred.

Accordingly, magenta coupler residues as Cp preferably include those represented by the formulae (III), (IV) and (V):



(III)

55



(IV)

60

wherein R<sub>1</sub> represents a nondiffusible group of from 8 to 32 total carbon atoms; and R<sub>2</sub>, which may be the same or different when R<sub>2</sub> represents two or more groups, represents one or more of a halogen atom, a lower alkyl group or a lower alkoxy group.

Specific examples of the colorless couplers are disclosed in, e.g., U.S. Pat. Nos. 3,912,513 and 4,204,867, and Japanese Patent Application (OPI) No. 152721/77, etc.



(V)

wherein R<sub>1</sub> represents a nondiffusible group having from 8 to 32 total carbon atoms; R<sub>2</sub> represents a halogen atom, a lower alkyl group, a lower alkoxy group, a phenyl group or a substituted phenyl group; and Z represents a non-metallic atomic group necessary to form a substituted or unsubstituted 5-membered azole ring containing from 2 to 4 nitrogen atoms (the substituent for the azole ring includes a condensed ring).

Typical examples of the cyan couplers are described in, e.g., U.S. Pat. Nos. 2,772,162, 2,895,826, 3,002,836, 3,034,892, 2,474,293, 2,423,730, 2,367,531 and 3,041,236, Japanese Patent Application (OPI) Nos. 99341/81, 155538/82, 204545/82, 189154/83, 31953/84, 118643/83, 187928/83 and 213748/83, and U.S. Pat. No. 4,333,999, etc. Of these, phenols and naphthols are preferred.

Accordingly, preferred cyan coupler residues as Cp include those having the following formulae (VI), (VII), (VIII) and (IX).



(VI)



(VII)



(VIII)



(IX)

Typical examples of these colorless couplers have skeletons represented by the following formulae (X), (XI) and (XII).



(X) 5

wherein R<sub>1</sub> represents a nondiffusible group of from 8 to 32 total carbon atoms; and R<sub>2</sub> represents a hydrogen atom, a halogen atom, a lower alkyl group or a lower alkoxy group.



(XI)

wherein R<sub>1</sub> represents a nondiffusible group of from 8 to 32 total carbon atoms; and V represents an oxygen atom, a sulfur atom or a nitrogen atom.



(XII)

wherein R<sub>1</sub> and R<sub>2</sub> each represents an alkoxy carbonyl group, an aminocarbonyl group, an acyl group, a group derived from a sulfonic acid or sulfonic acid derivative corresponding to the above described groups, a cyano group, an ammonium group, a nitrogen-containing heterocyclic group which is bonded at the N-position thereof, or a like group; R<sub>1</sub> and R<sub>2</sub> may be bonded together to form a 5- or 6-membered ring.

Cp further includes coupler residues of couplers which form a black color upon reacting with an oxidation product of a developing agent. Examples of such black color forming couplers are described in, e.g., U.S. Pat. Nos. 1,939,231, 2,181,944, 2,333,106 and 4,126,461, West German Patent Application (OLS) Nos. 2,644,194 and 2,650,764, etc.

More specifically, these black color forming couplers are represented by the following formulae (XIII), (XIV) and (XV).



(XIII)



(XIV)

65



(XV)

8

-continued

5

- 10 wherein R<sub>1</sub> represents an alkyl group of from 3 to 20 carbon atoms, a phenyl group, or a phenyl group substituted with a hydroxyl group, a halogen atom, an amino group or an alkyl or alkoxy group of from 1 to 20 carbon atoms; R<sub>2</sub>'s, which may be the same or different, 15 represent a hydrogen atom, a halogen atom, an alkyl or alkenyl group of from 1 to 20 carbon atoms or an aryl group of from 6 to 20 carbon atoms; and R<sub>3</sub>, which may be the same or different when R<sub>3</sub> represents two or more groups, represents one or more of a halogen atom, 20 an alkyl or alkoxy group of from 1 to 20 carbon atoms or any other monovalent organic group.

Cp as represented by the above described formulae (I) to (XV) may form a polymer including a dimer, a trimer, etc., at the moiety other than the coupling position, and may also be bonded to a polymer at the moiety other than the coupling position.

In the formula (2), the coupler residues as represented by Cp have partial structures represented by the aforementioned formulae (I) to (XV), wherein the asterisk (\*) indicates a position to which BALL is bonded and  $-(TIME)_n-FA$  is bonded to one of other positions.

In the formula (2), the nondiffusible group as represented by BALL has such a size and a form that impart nondiffusibility to couplers. The nondiffusible group 35 may be a polymeric group comprising a plurality of releasable groups connected to each other, or may have a nondiffusibility-imparting alkyl and/or aryl group(s). In the latter case, the alkyl and/or aryl group(s) preferably contain(s) about 8 to 32 total carbon atoms. BALL 40 has a group for bonding to the coupling position of Cp. Such a group for bonding typically includes  $-O-$ ,  $-S-$ ,  $-N=N-$ ,



that constitutes a heterocyclic ring.

In the formula (3), the group represented by RED is a group having a skeleton of hydroquinone, catechol, o-aminophenol or p-aminophenol and capable of undergoing oxidation-reduction reaction with an oxidation product of an aromatic primary amine developing agent and subsequently alkali-hydrolysis to thereby release  $-(TIME)_n-FA$ . In the hereinafter given formulae (XVI) to (XXI), the group  $-(TIME)_n-FA$  is abbreviated as FR.

Specific examples of RED are represented by the following formulae (XVI) to (XXI).



(XVI)

-continued



wherein R<sub>1</sub> represents a hydrogen atom, a halogen atom, an alkyl group, an aryl group, an alkoxy group, an aryloxy group, an alkylthio group, an arylthio group, a cyano group, an alkoxy carbonyl group, a carbamoyl group, a sulfamoyl group, a carboxyl group, a sulfo group, a sulfonyl group, an acyl group, a carbonamido group, a sulfonamido group or a heterocyclic group; when R<sub>1</sub> represents two or more groups, they may be the same or different, or two vicinal R<sub>1</sub> groups may be connected to form a benzene ring or a 5- to 7-membered hetero ring; R<sub>2</sub> represents an alkyl group, an aryl group, an acyl group, a carbamoyl group, a sulfonyl group or a sulfamoyl group; and T<sub>1</sub>, which may be the same or different in the formulae (XVI) or (XVII), represents a hydrogen atom or a group releasable by hydrolysis under an alkaline condition.

Typical examples of T<sub>1</sub> include a hydrogen atom, an acyl group, a sulfonyl group, an alkoxy carbonyl group, a carbamoyl group, an oxaryl group, etc.

The timing group as represented by TIME can include a group which is releasable from Cp or RED by coupling reaction or oxidation-reduction reaction and then releases FA through intramolecular substitution as described in, e.g., U.S. Pat. No. 4,248,962 and Japanese Patent Application (OPI) No. 56837/82; a group which releases FA by electron transfer reaction via a conjugated system as described in, e.g., British Pat. No. 2,072,363 A and Japanese Patent Application (OPI) Nos. 154234/82, 188035/82, 114946/81, 56837/82, 209736/83, 209727/83, 209738/83, 209740/83 and 98728/83; and a group which releases FA by coupling

(XVII) 5 reaction with an oxidation product of an aromatic primary amine developing agent as described in, e.g., Japanese Patent Application (OPI) No. 111536/82. These reactions may be completed in one step or in multiple steps.

(XVIII) 10 Further, the trivalent TIME group which is bonded to the coupling position and non-coupling position of Cp and FA as hereinbefore described is also preferred. Examples of such a trivalent TIME group is disclosed in Japanese Patent Application (OPI) No. 209740/83 in which TIME is incorporated in a yellow coupler.

(XIX) 15 When FA contains AD-(L)<sub>m</sub>-X, AD may be directly bonded to a carbon atom of the coupling position, or either L or X, if releasable upon coupling reaction, 15 may be bonded to the coupling carbon atom. Further, a so-called 2-equivalent coupling-off group may be present between the coupling carbon and AD.

(XX) 20 These FA groups can include an alkoxy group (e.g., a methoxy group), an aryloxy group (e.g., a phenoxy group), an alkylthio group (e.g., an ethylthio group), an arylthio group (e.g., a phenylthio group), a heterocyclic oxy group (e.g., a tetrazolyl group), a heterocyclic thio group (e.g., a pyridylthio group), a heterocyclic group (e.g., a hydantoinyl group, a pyrazolyl group, a 25 triazolyl group, a benzotriazolyl group, etc.), and the like. In addition, those described in British Pat. No. 2,011,391 can also be used as FA.

(XXI) 30 The group adsorptive onto silver halide grains as represented by AD can include a group derived from a nitrogen-containing heterocyclic ring having a dissociative hydrogen atom (e.g., pyrrole, imidazole, pyrazole, triazole, tetrazole, benzimidazole, benzopyrazole, benzotriazole, uracil, tetraazaindene, imidazotetrazole, pyrazolotriazole, pentaazaindene, etc.), a heterocyclic ring containing at least one nitrogen atom and other hetero atoms (e.g., an oxygen atom, a sulfur atom, a selenium atom, etc.) (e.g., oxazole, thiazole, thiazoline, thiazolidine, thiadiazole, benzothiazole, benzoxazole, benzoselenazole, etc.), a heterocyclic ring having a mercapto group (e.g., 2-mercaptopbenzothiazole, 2-mercaptopurine, 2-mercaptopbenzoxazole, 1-phenyl-5-mercaptotetrazole, etc.), a quaternary salt (e.g., quaternary salts of tertiary amine, pyridine, quinoline, benzothiazole, benzimidazole or benzoxazole, etc.), a thiophenol, an alkylthiol (e.g., cysteine), and a compound having a partial structure of



(e.g., thiourea, dithiocarbamate, thioamide, rhodanine, thiazolidinethione, thiohydantoin, thiobarbituric acid, etc.).

(XVI) 60 The divalent linking group as represented by L in FA is composed of a group selected from an alkylene group, an alkylene group, a phenylene group, a naphthylene group, —O—, —S—, —SO—, —SO<sub>2</sub>—, —N=N—, a carbonyl group, an amido group, a thioamido group, a sulfonamido group, a ureido group, a thioureido group, a heterocyclic group, etc. If a group capable of being cleaved by the action of a component of a developing solution, such as hydroxide ions, hydroxylamine, sulfite ions, etc., is selected as one of the divalent linking groups which constitute L, the fogging activity can be controlled or deactivated.

The group as represented by X can include groups derived from reducing compounds (e.g., hydrazine,

hydrazide, hydrazone, hydroquinone, catechol, p-aminophenol, p-phenylenediamine, 1-phenyl-3-pyrazolidone, enamine, aldehyde, polyamine, acetylene, aminoboran, a quaternary salt such as a tetrazolium salt and an ethylene-bispyridinium salt, carbazic acid, etc.) and groups derived from compounds capable of forming silver sulfide upon development, such as compounds having a partial structure of



(e.g., thiourea, thioamide, dithiocarbamate, rhodanine, thiohydrantoin, thiazolidinethione, etc.). Of these groups, some of those capable of forming silver sulfide upon development have adsorptivity onto silver halide grains and, therefore, can serve as AD.

Particularly preferred FA can be represented by the following formulae (XXII) and (XXIII).



(XXII)



(XXIII)

wherein  $R_1$  represents an acyl group (e.g., a formyl group, an acetyl group, a propionyl group, a trifluoroacetyl group, a pyruvoyl group, etc.), a carbamoyl group (e.g., a dimethylcarbamoyl group, etc.), an alkylsulfonyl group (e.g., a methanesulfonyl group, etc.), an arylsulfonyl group (e.g., a benzenesulfonyl group, etc.), an alkoxy carbonyl group (e.g., a methoxycarbonyl group, etc.), an aryloxycarbonyl group (e.g., a phenoxy carbonyl group, etc.) or a sulfamoyl group (e.g., a methylsulfamoyl group, etc.);  $R_2$  represents a hydrogen atom, an acyl group (e.g., a trifluoroacetyl group, etc.), an alkoxy carbonyl group (e.g., a methoxycarbonyl group, etc.) or an aryloxycarbonyl group (e.g., a phenoxy carbonyl group, etc.);  $R_3$  represents a halogen atom (e.g., a fluorine atom, a chlorine atom, etc.), an alkoxy group (e.g., a methoxy group, a methoxyethoxy group, etc.), an alkyl group (e.g., a methyl group, a hydroxymethyl group, etc.), an alkenyl group (e.g., an allyl group, etc.), an aryl group (e.g., a phenyl group, etc.), an aryloxy group (e.g., a phenoxy group, etc.), an alkylthio group (e.g., a methylthio group, etc.), an arylthio group (e.g., a phenylthio group, etc.), a carbonamido group (e.g., an acetamido group, etc.) or a sulfonamido group (e.g., a methanesulfonamido group, etc.);  $m$  represents 0 or an integer of from 1 to 4; when  $m$  is 2 or more,  $R_3$  may be the same or different or two or more of them may be taken together to form a condensed ring;  $L$  is a divalent group as defined above;  $n$  represents 0 or 1;  $Z_1$  represents a monocyclic or condensed hetero ring; and  $Z_2$  represents an atomic group

necessary to form a monocyclic or condensed ring together with the



In the formulae (XXII) and (XXIII), specific examples of the monocyclic or condensed hetero rings formed by



will be shown in examples of AD hereinafter given.

Examples of FR compounds which can be used in the present invention are described in, e.g., Japanese Patent Application (OPI) Nos. 150845/82, 50439/84, 177638/84 and 170840/84.

Specific examples of AD are shown below. In the following formulae, the free bonds are bonded to  $-(L)_m-X$  and  $-(TIME)_n-$ .



-continued



Specific examples of L are shown below.

—CH<sub>2</sub>—, —CH<sub>2</sub>CH<sub>2</sub>—, —OCH<sub>2</sub>—, —OCH<sub>2</sub>CH<sub>2</sub>—, 65  
 —SCH<sub>2</sub>—, —COO—,

**15**

-continued

**16**

-continued



-continued



-continued



Specific examples of preferred FA groups in the aforesaid formulae (1) to (3) are shown below.



Specific examples of the compounds which can be used in the present invention are shown below.



-continued



-continued



-continued



(I-19)



(I-20)



(I-21)



(I-22)



(I-23)

4,656,123

27

28

-continued

(I-24)



(I-25)



(I-26)



(I-27)



-continued

(I-28)



(II-1)



(II-2)



(II-3)



(II-4)

(II-5)



(II-6)



(II-7)



(II-8)

(III-1)



-continued



-continued

(III-7)



(III-8)



(III-9)



(III-10)



These FR-releasing compounds of the present invention can be synthesized from generally known compounds by the methods described, e.g., in Japanese Patent Application (OPI) Nos. 150845/82 and 138636/82, U.S. Pat. Nos. 3,214,377 and 3,253,924 and Japanese Patent Application Nos. 161515/82, 45 146097/83 and 214808/83, etc.

The FR-releasing compound is used in an amount ranging from  $1 \times 10^{-8}$  to 0.5 mols, and preferably from  $5 \times 10^{-7}$  to  $1 \times 10^{-2}$  mols, per mol of a silver halide 50 light-sensitive emulsion in which the FR-compound is to be incorporated.

Silver halides which are not substantially developed (hereinafter referred to as "non-developable silver halides") in accordance with the present invention are 55 silver halide grains which are not substantially developed when a light-sensitive material containing such silver halide grains is exposed to an adequate amount of light and then processed under ordinary development conditions. Further, while the development accelerator of the present invention exerts its activity upon acting 60 on silver halides in a light-sensitive layer by development processing; the non-developable silver halide grains in a layer outside of said light-sensitive layer are not substantially developed even after the manifestation 65 of the development accelerator.

The non-developable silver halide grains which can be used in the present invention are not limited to any particular halogen component(s), and include those

such as silver chloride, silver bromide, silver iodide, silver chlorobromide, silver iodobromide and silver chloroiodobromide. However, silver halide grains having a silver bromide content of 60 mol% or more, a silver chloride content of 30 mol% or less, and a silver iodide content of 40 mol% or less, are preferred. Silver iodobromide containing from 0 to about 20 mol% of silver iodide is more preferred in view of low developability. The most preferred is silver iodobromide containing from 0.3 to about 5 mol% of silver iodide from the standpoint that light absorption of silver halide grains in the visible region is not increased.

It is preferable that the non-developable silver halide grains according to the present invention have a relatively small grain size in view of low light-sensitivity and less absorption in a visible region. The mean grain size is preferably not more than about 0.2  $\mu$ m, more preferably not more than 0.15  $\mu$ m, and most preferably not more than 0.10  $\mu$ m. In the following description, the non-developable silver halide grains having a mean grain size of not more than about 0.2  $\mu$ m will be referred to as "fine silver halide grains" or more simply as "fine grains".

The non-developable silver halide emulsion which can be used in the present invention may have an arbitrary grain size distribution, but narrow grain size distribution is preferred. In particular, it is more preferred

that the size range of 90% of the weight of the total silver halide grains falls within  $\pm 40\%$  of the mean grain size.

The fine silver halide grains which can be used in the present invention can be prepared by using known methods, e.g., the acid process, the neutral process, the ammonia process, and the like. The reaction between a soluble silver salt and a soluble halogen salt can be carried out by any of a single jet method, a double jet method or a combination thereof. The so-called controlled double jet method, in which the pAg of a liquid phase wherein silver halide is formed is maintained constant, can also be employed. This method is advantageous since the resulting silver halide grains have narrow size distribution.

The fine silver halide grains may have a regular crystal form, such as cubic, octahedral, dodecahedral, tetradecahedral, etc., or an irregular crystal form, such as spherical, plate-like, etc. The individual emulsion grains may comprise a core and an outer shell having different halogen compositions, or may be homogeneous. The fine grain emulsion may contain impurities, such as cadmium ions, lead ions, iridium ions, rhodium ions, and the like. Fine grains containing a desensitizer, such as rhodium, in the interior thereof are preferred. The fine grains may be either a surface latent image type or an internal latent image type, and they may contain a fog nucleus in the interior thereof. The internal latent image type silver halide grains can be used to advantage as non-developable silver halide in the present invention because of their non-susceptibility to development with commonly employed surface developers.

The fine grain emulsion may be subjected to conventional chemical sensitization, i.e., sulfur sensitization, gold sensitization, reduction sensitization or a combination thereof. However, it is preferable to use a so-called primitive emulsion that has not been subjected to chemical sensitization.

The fine grain emulsion can contain various dyes, such as cyanine dyes, merocyanine dyes, complex cyanine dyes, complex merocyanine dyes, holopolar cyanine dyes, hemicyanine dyes, styrene dyes, hemioxonol dyes, and the like. Desensitizing dyes that are unfavorable in usual negatively-working emulsions due to their high desensitizing property can also be used in the present invention to advantage. The fine grain emulsion can further contain antifoggants or stabilizers, such as azoles, heterocyclic compounds, mercapto compounds, thioketo compounds, azaindenes, benzenethiosulfonic acids, benzenesulfonic acids, and the like.

The non-developable silver halide emulsion of the present invention generally is used in an amount of from 0.002 to 2 g/m<sup>2</sup> (silver coverage), and is preferably used in an amount of from 0.01 to 1 g/m<sup>2</sup> (silver coverage). Binders for the non-developable silver halide-containing layer include conventional hydrophilic polymers, and preferably gelatin. The amount of the binder to be used is preferably less than 250 g per mol of silver halides.

The non-developable fine silver halide emulsion is applied between a color-sensitive emulsion layer containing the FR-releasing compound and a layer differing in color sensitivity. In light-sensitive materials containing a development inhibitor-releasing compound in the light-sensitive layer thereof, it is known in the art to provide a fine grain emulsion layer between emulsion layers having different color sensitivities for the purpose of controlling diffusion of a development inhibitor re-

leased upon development from a certain light-sensitive emulsion layer into another emulsion layer having a different color sensitivity. This conventional technique takes advantage of the physical adsorption of the development inhibitor onto silver halide grains. On the other hand, in the present invention, it is believed that the FR compound released from the FR-releasing compound undergoes a chemical reaction with the non-developable silver halides, such as electron donation, and is thereby deactivated. This concept is supported by experimental results showing that FR compounds like II-2 having no adsorbing group can be deactivated by the non-developable silver halides.

In the case when three kinds of emulsions A, B, and C having different color sensitivities from each other are provided on a support in the order listed above and the emulsion A contains an FR-releasing compound, the non-developable silver halide grains may be present in either one or both of insensitive intermediate layers provided between A and B and between B and C. It is preferable to incorporate the non-developable silver halide in an insensitive intermediate layer interposed between an emulsion layer containing an FR-releasing compound and the adjacent emulsion layer having color sensitivity different from that of the FR-releasing compound-containing layer. Taking the above-described example wherein the emulsion A contains an FR-releasing compound, the non-developable silver halide is preferably present between the emulsions A and B. When the emulsion B contains an FR-releasing compound, the object of the present invention can be achieved by incorporating the non-developable silver halide in either one of, and preferably both, of the intermediate layer between A and B and the intermediate layer between B and C. In another embodiment in which the emulsion A or C contains an FR-releasing compound, the non-developable silver halide can be incorporated in the emulsion B.

The light-sensitive layer containing an FR-releasing compound according to the present invention may have two or more emulsion layers that differ in sensitivity but are sensitive to the same color, e.g., a combination of a high sensitive emulsion layer and a low sensitive emulsion layer.

These two or more silver halide emulsion layers having substantially the same color sensitivity different sensitivities may or may not be adjacent to each other. It is sufficient that the FR-releasing compound be present in at least one of these layers, but the FR-releasing compound is preferably present in the most sensitive layer.

Layer structures of light-sensitive materials having at least two emulsion layers being sensitive to the same color but different in sensitivity include various embodiments. Some examples are described in *Research Disclosure*, No. 22534 (Jan., 1983). As shown in the specific examples given in this literature, emulsions in which at least 50% of the total projection area of the total silver halide grains is occupied by plate-like silver halide grains each having a grain diameter 5 times or more its thickness can be employed. Further, the object of this invention can be accomplished by incorporating the non-developable silver halide emulsion of the present invention in an intermediate layer, which is preferably insensitive, present between an emulsion layer containing an FR-releasing compound and the adjacent emulsion layer differing in color sensitivity.

The compounds or couplers according to the present invention can be incorporated in silver halide emulsion layers by known methods as described, e.g., in U.S. Pat. No. 2,322,027. For example, the compound is dissolved in a high-boiling organic solvent, such as an alkyl phthalate (e.g., dibutyl phthalate, diethyl phthalate, etc.), a phosphoric ester (e.g., diphenyl phosphate, triphenyl phosphate, tricresyl phosphate, diethylbutyl phosphate, etc.), a citric ester (e.g., tributyl acetylacetate, etc.), a benzoic ester (e.g., octyl benzoate, etc.), an alkylamide (e.g., diethyllaurylamine, etc.), a fatty acid ester (e.g., dibutoxyethyl succinate, diethyl azelate, etc.), a trimesic ester (e.g., tributyl trimesate, etc.), etc., or an organic solvent having a boiling point of from about 30° to 150° C., such as a lower alkyl acetate (e.g., ethyl acetate, butyl acetate, etc.), ethyl propionate, sec-butyl alcohol, methyl isobutyl ketone,  $\beta$ -ethoxyethyl acetate, methyl cellosolve acetate, etc., or a mixture of these high-boiling point solvents and low-boiling point solvents, and the resulting solution is dispersed in a hydrophilic colloid.

The dispersion method using a polymer as described in Japanese Patent Publication No. 39850/76 and Japanese Patent Application (OPI) No. 59943/76 can also be employed for the incorporation of the compounds according to the present invention.

When the compound or coupler according to the present invention has an acid group, e.g., a carboxyl group, a sulfo group, etc., it can be incorporated into a hydrophilic colloid as an alkaline aqueous solution thereof.

The photographic emulsion layers of the light-sensitive materials according to the present invention can contain conventional color forming couplers, i.e., compounds capable of forming colors upon oxidative coupling with aromatic primary amine developing agents (e.g., phenylenediamine derivatives, aminophenol derivatives, etc.) in color development processing, in combination with the FR-releasing compounds of the present invention. Examples of the magenta couplers which can be used include 5-pyrazolone couplers, pyrazolobenzimidazole couplers, cyanoacetylumone couplers, open-chain acylacetone nitrile couplers, and the like. Examples of conventional yellow couplers include acylacetamide couplers (e.g., benzoyl acetanilides, pivaloyl acetanilides, etc.), and the like. Examples of conventional cyan couplers include naphthol couplers, phenol couplers, and the like. It is desirable that these couplers have hydrophobic groups called ballast groups in their molecules and are thereby rendered non-diffusible; alternatively, the couplers can have a polymeric structure. These couplers may be 4-equivalent or 2-equivalent with respect to silver ions. Moreover, they may be colored couplers having a color correcting effect.

The light-sensitive materials may contain two or more of the above-described couplers and the like in one layer thereof, or one of these couplers may be incorporated into two or more layers, in order to meet characteristic requirements for the light-sensitive materials.

Photographic color forming couplers to be used can be advantageously selected so as to give a middle-scaled image. It is preferable that cyan dyes formed from cyan couplers have a maximum absorption band between about 600 and about 720 nm; magenta dyes formed from magenta couplers have a maximum absorption band between about 500 and about 580 nm; and yellow dyes

formed from yellow couplers have a maximum absorption band between about 400 and about 480 nm.

Binders or protective colloids which can be used in the emulsion layers or intermediate layers of the light-sensitive materials preferably include gelatin, but other hydrophilic colloids may also be used.

Silver halides of photographic emulsion layers which can be used in the light-sensitive materials according to the present invention may be any of silver bromide, silver iodobromide, silver iodochlorobromide, silver chlorobromide and silver chloride. Silver halide emulsions having a silver bromide content of 60 mol% or more, a silver chloride content of 30 mol% or less, and a silver iodide content of 40 mol% or less are useful. The more preferred are silver iodobromide emulsions having a silver iodide content of from 2 to 25 mol%, with those having a silver iodide content of from 8 to 25 mol% being the most preferred.

A mean grain size of silver halide grains in the photographic light-sensitive emulsions (the grain size being defined as grain diameter if the grain has a spherical or a nearly spherical form and as a length of the edge if the grain has a cubic form, and being averaged based on projected areas of the total grains) is not particularly restricted. However, the emulsion to be used in the layer containing the FR-releasing compound of the present invention preferably has a mean grain size of not less than 0.6  $\mu$ m, more preferably not less than 1.0  $\mu$ m, and most preferably not less than 1.5  $\mu$ m. Grain size distribution may be either narrow or broad.

Light-sensitive silver halide grains in the photographic emulsion may have a regular crystal form, such as cubic, octahedral, etc., an irregular crystal form, such as spherical, plate-like, etc., or a composite form thereof. Silver halide grains may be a mixture of grains having various crystal forms.

Further, an emulsion in which a plate-like silver halide grain having a diameter 5 times or more its thickness occupies 50% or more of the total projection area may also be employed.

The individual light-sensitive silver halide grains may have a so-called core-shell structure having different halogen compositions between the inside and surface thereof. In addition, they may be grains wherein a latent image is predominantly formed on their surface, or may be grains where a latent image is predominantly formed in the interior thereof.

Two or more light-sensitive silver halide emulsions which have been separately prepared can be used as a mixture.

In a process for producing light-sensitive silver halide grains or physical ripening of the produced grains, cadmium salts, zinc salts, lead salts, thallium salts, iridium salts or complex salts thereof, rhodium salts or complex salts thereof, iron salts or complex salts thereof, and the like may be present.

After the formation of silver halide grains or the physical ripening of the grains, soluble salts are usually removed from the emulsion by, for example, a conventionally known noodle washing method comprising gelling the gelatin, or a sedimentation (flocculation) method using an inorganic salt composed of a polyvalent anion (e.g., sodium sulfate), an anionic surface active agent, an anionic polymer (e.g., polystyrenesulfonic acid) or a gelatin derivative (e.g., aliphatic acylated gelatin, aromatic acylated gelatin or aromatic acylated gelatin).

The light-sensitive silver halide emulsion is usually subjected to chemical sensitization. Chemical sensitization can be carried out using processes as described in, e.g., H. Frieser (ed.), *Die Grundlagen der Photographischen Prozesse mit Silberhalogeniden*, 675-734, Akademische Verlagsgesellschaft (1968).

More specifically, chemical sensitization can be achieved by sulfur sensitization using compounds containing sulfur capable of reacting with active gelatin or silver ions (e.g., thiosulfates, thioureas, mercapto compounds, rhodanines, etc.); reduction sensitization using reducing materials (e.g., stannous salts, amines, hydrazines, formamidinesulfonic acid, silane compounds, etc.); noble metal sensitization using noble metal compounds (e.g., gold complexes, and complexes of Periodic Table Group VIII metals such as Pt, Ir, Pd, etc.); and the like, individually, or in combinations thereof.

Photographic light-sensitive emulsions used in the present invention can contain various compounds for the purpose of preventing fog in the preparation, storage, photographic processing, or stabilizing photographic properties. Specific examples of such compounds include azoles, such as benzothiazolium salts, nitroimidazoles, nitrobenzimidazoles, chlorobenzimidazoles, bromobenzimidazoles, mercaptobenzimidazoles, mercaptobenzothiazoles, mercaptobenzimidazoles, mercaptothiadiazoles, aminotriazoles, benzotriazoles, nitrobenzotriazoles, mercaptotetrazoles (particularly 1-phenyl-5-mercaptotetrazole), etc.; mercaptopyrimidines; mercaptotriazines; thioketo compounds, such as oxazolinethione, etc.; azaindenes, such as triazaindenes, tetraazaindenes (particularly 4-hydroxy-substituted (1,3,3a,7)tetraazaindenes), pentaazaindenes, etc.; benzethiosulfonic acid; benzenesulfonic acid; benzenesulfonic acid amide; and other various compounds known as anti-foggants or stabilizers.

For details of specific examples and usages of these compounds, disclosures in, e.g., U.S. Pat. Nos. 3,954,474 and 3,982,947, and Japanese Patent Publication No. 28660/77 can be referred to.

Specific examples of surface active agents which can be used include nonionic surface active agents, such as saponin (steroid type), alkylene oxide derivatives (e.g., polyethylene glycol, polyethylene glycol/polypropylene glycol condensates, polyethylene glycol alkyl ethers or alkyl aryl ethers, polyethylene glycol esters, polyethylene glycol sorbitan esters, polyalkylene glycol alkylamines or alkylamides, polyethylene oxide adducts of silicone, etc.), glycidol derivatives (e.g., alkenylsuccinic polyglycerides, alkylphenol polyglycerides, etc.), fatty acid esters of polyhydric alcohols, alkyl esters of sugars, and the like; anionic surface active agents containing acidic groups, e.g., a carboxyl group, a sulfo group, a phospho group, a sulfuric ester group, a phosphoric ester group, etc., such as alkylcarboxylates, alkylsulfonates, alkylbenzenesulfonates, alkylnaphthalenesulfonates, alkylsulfates, alkylphosphates, N-acyl-N-alkyltaurines, sulfosuccinates, sulfoalkylpolyoxyethylene alkyl phenyl ethers, polyoxyethylene alkylphosphates, and the like; amphoteric surface active agents, such as amino acids, aminoalkylsulfonic acids, aminoalkyl sulfates or phosphates, alkylbetaines, amine oxides and the like; and cationic surface active agents, such as alkylamine salts, aliphatic or aromatic quaternary ammonium salts, heterocyclic quaternary ammonium salts (e.g., pyridinium, imidazolium, etc.), aliphatic or heterocyclic phosphonium or sulfonium salts, and the like.

The photographic emulsions of the photographic light-sensitive materials according to the present invention may contain, for example, polyalkylene oxides or derivatives thereof (e.g., ethers, esters and amines thereof), thioether compounds, thiomorpholines, quaternary ammonium salt compounds, urethane derivatives, urea derivatives, imidazole derivatives, 3-pyrazolidones, and the like for the purpose of increasing sensitivity or contrast or accelerating development. Examples of such compounds are disclosed, e.g., in U.S. Pat. Nos. 2,400,532, 2,423,549, 2,716,062, 3,617,280, 3,772,021 and 3,808,003, British Pat. No. 1,488,992, etc.

The photographic emulsion layers or other hydrophilic colloidal layers of the light-sensitive materials of the present invention can further contain dispersions of water-insoluble or slightly soluble synthetic polymers for the purpose of improving dimensional stability and so on. Such polymers include those having, as monomer components, one or more of alkyl (meth)acrylates, alkoxalkyl, (meth)acrylates, glycidyl (meth)acrylate, (meth)acrylamide, vinyl esters (e.g., vinyl acetate), acrylonitrile, olefins and styrene, or a combination of these monomers and acrylic acid, methacrylic acid, an  $\alpha,\beta$ -unsaturated dicarboxylic acid, a hydroxyalkyl (meth)acrylate, a sulfoalkyl (meth)acrylate, styrenesulfonic acid, etc.

Any of conventional methods and processing solutions as described, e.g., in *Research Disclosure*, No. 176, 28-30, can be applied to photographic processing of the light-sensitive materials according to the present invention. Any photographic processing, whether for the formation of silver images (achromatic photographic processing) or for the formation of dye images (color photographic processing), can be used depending on the intended end use of the light-sensitive material. Processing temperatures are generally selected from 18° to 50° C., but temperatures outside of this range may also be used. However, the light-sensitive materials having the non-developable silver halide layer according to the present invention can exert its conspicuous effect particularly when developed at a high temperature of 30° C. or more. In addition, the light-sensitive materials according to the present invention can effectively be employed in a continuous processing system using a replenisher.

For development processing, a method where a developing agent is contained in the light-sensitive material, e.g., in an emulsion layer, and the light-sensitive material is treated in an aqueous alkaline solution to effect development may be employed. Developing agents which are hydrophobic can be incorporated in emulsion layers using various methods as described, e.g., in *Research Disclosure*, No. 169 (RD-16928), U.S. Pat. No. 2,739,890, British Pat. No. 813,253, West German Pat. No. 1,547,763, etc. Such development processing may be carried out in combination with silver salt stabilizing processing using a thiocyanate.

A conventional fixing solution can be employed. Examples of fixing agents which can be used include not only thiosulfates and thiocyanates, but also organic sulfur compounds which are known to have a fixing effect. The fixing solution may contain a water-soluble aluminum salt as a hardener.

Dye images can be formed in accordance with conventional methods, for example, the negative-positive method as described, e.g., in *Journal of the Society of Motion Picture and Television Engineers*, vol. 61, 667-701 (1953).

Developing solutions which can be used for achromatic photographic processing can contain conventionally known developing agents. Examples of such developing agents include dihydroxybenzenes (e.g., hydroquinone), 3-pyrazolidones (e.g., 1-phenyl-3-pyrazolidone), aminophenols (e.g., N-methyl-p-aminophenol), ascorbic acid, etc. or combinations thereof. The developing solution generally contains known preservatives, alkali agents, pH buffers, antifoggants, and the like, and may further contain, if desired, dissolution assistants, color toning agents, development accelerators, surface active agents, defoaming agents, water softeners, hardeners, viscosity-imparting agents, and the like.

Color developing solutions which can be used for color photographic processing generally comprise an alkaline aqueous solution containing a color developing agent. Specific examples of the color developing agents include known aromatic primary amine developers, such as phenylenediamines (e.g., 4-amino-N,N-diethylaniline, 3-methyl-4-amino-N,N-diethylaniline, 4-amino-N-ethyl-N-β-hydroxyethylaniline, 3-methyl-4-amino-N-ethyl-N-β-hydroxyethylaniline, 3-methyl-4-amino-N-ethyl-N-β-methanesulfoamidoethylaniline, 4-amino-3-methyl-N-ethyl-N-β-methoxyethylaniline, etc.).

In addition to the above-described color developing agents, those described in L. F. A., Mason, *Photographic Processing Chemistry*, 226-229, Focal Press (1966), U.S. Pat. Nos. 2,193,015 and 2,592,364, Japanese Patent Application (OPI) No. 64933/73, etc., may also be employed.

The color developing solution can additionally contain a pH buffer, e.g., a sulfite, carbonate, borate or phosphate of an alkali metal, a development inhibitor or antifoggant, e.g., a bromide, an iodide, an organic antifoggant, etc. If desired, it may further contain a water softener, a preservative (e.g., hydroxylamine), an organic solvent (e.g., benzyl alcohol, diethylene glycol, etc.), a development accelerator (e.g., polyethylene glycol, quaternary ammonium salts, amines, etc.), a color forming coupler, a competing coupler, a fogging agent (e.g., sodium boron hydride), an assistant developer (e.g., 1-phenyl-3-pyrazolidone), a viscosity-imparting agent, a polycarboxylic acid series chelating agent, an antioxidant, and the like. Specific examples of these additives are disclosed, e.g., in *Research Disclosure*, No. 176 (RD-17643), U.S. Pat. No. 4,083,723, West German Patent Application (OLS) No. 2,622,950, etc.

After color development, the photographic emulsion is generally subjected to a conventional bleaching treatment. Bleaching may be carried out simultaneously with fixing, or these two processes may be carried out separately. Bleaching agents which can be used include, for example, compounds of polyvalent metals, such as iron (III), cobalt (III), chromium (IV), copper (II), etc., peroxy acids, quinones, nitroso compounds, and the like. More specifically, useful bleaching agents include ferricyanides; bichromates; complex salts formed by iron (III) or cobalt (III) and aminopolycarboxylic acids, e.g., ethylenediaminetetraacetic acid, nitrilotriacetic acid, 1,3-diamino-2-propanoltetraacetic acid, etc., or organic acids, e.g., citric acid, tartaric acid, malic acid, etc.; persulfates; permanganates; nitrosophenol; and the like. Of these, potassium ferricyanide, sodium(ethylenediaminetetraacetato)ferrate (III), and ammonium(ethylenediaminetetraacetato)ferrate (III) are particularly useful. The (ethylenediaminetetraacetato)iron

(III) complexes are useful in either an independent bleaching solution or a combined bleach-fix solution.

The bleaching or bleach-fix bath can contain a bleach accelerating agent as described in U.S. Pat. Nos. 3,042,520 and 3,241,966, Japanese Patent Publication Nos. 8506/70 and 8836/70, etc., thiol compounds as described in Japanese Patent Application (OPI) No. 65732/78, and various other conventional additives.

Photographic light-sensitive emulsions employed in the present invention may be spectrally sensitized with methine dyes and others. Sensitizing dyes which can be used for spectral sensitization include cyanine dyes, merocyanine dyes, complex cyanine dyes, complex merocyanine dyes, holopolar cyanine dyes, hemicyanine dyes, styryl dyes and hemioxonol dyes. Of these, cyanine dyes, merocyanine dyes and complex merocyanine dyes are particularly useful. Any nuclei commonly used for cyanine dyes as basic heterocyclic nuclei can be applied to the above-described dyes. Specific examples of such nuclei include a pyrrolidine nucleus, an oxazoline nucleus, a thiazoline nucleus, a pyrrole nucleus, an oxazole nucleus, a thiazole nucleus, a selenazole nucleus, an imidazole nucleus, a tetrazole nucleus, a pyridine nucleus, etc.; the above-recited nuclei to which an alicyclic hydrocarbon ring is fused; and the above-recited nuclei to which an aromatic hydrocarbon ring is fused, i.e., an indolenine nucleus, a benzindolenine nucleus, an indole nucleus, a benzoxazole nucleus, a naphthoxazole nucleus, a benzothiazole nucleus, a naphthothiazole nucleus, a benzoselenazole nucleus, a benzimidazole nucleus, a quinone nucleus, etc. These nuclei may be substituted at their carbon atoms.

The merocyanine dyes or complex merocyanine dyes can have a 5- to 6-membered heterocyclic nucleus as a nucleus having a ketomethylene structure, such as a pyrazolin-5-one nucleus, a thiohydantoin nucleus, a 2-thioxazolidine-2,4-dione nucleus, a thiazolidine-2,4-dione nucleus, a rhodanine nucleus, a thiobarbituric acid nucleus, etc.

These sensitizing dyes can be used alone or in combinations thereof. Combinations of sensitizing dyes are frequently employed for the purpose of supersensitization. Typical examples of supersensitizing combinations are described in U.S. Pat. Nos. 2,688,545, 2,977,229, 3,397,060, 3,522,052, 3,527,641, 3,617,293, 3,628,964, 3,666,480, 3,672,898, 3,679,428, 3,703,377, 3,769,301, 3,814,609, 3,837,862 and 4,026,707, British Pat. Nos. 1,344,281 and 1,507,803, Japanese Patent Application Nos. 4936/68 and 12375/78 and Japanese Patent Application (OPI) Nos. 110618/77 and 109925/77, etc.

The photographic emulsions may also contain compounds which do not exhibit per se any spectral sensitizing activity or do not substantially absorb visible light, but which exhibit a supersensitizing activity when used in combination with the above-described sensitizing dyes. Such compounds include, for example, aminostyryl compounds as described, e.g., in U.S. Pat. Nos. 2,933,390 and 3,635,721, aromatic organic acid-formaldehyde condensates as described, e.g., in U.S. Pat. No. 3,743,510, cadmium salts, azaindene compounds, and the like. Combinations disclosed in U.S. Pat. Nos. 3,615,613, 3,615,641, 3,617,295 and 3,635,721 are particularly useful.

The present invention can be applied to a multilayer multicolor photographic material comprising a support having provided thereon at least two layers having different spectral sensitivities. A multilayer color photographic material usually has at least one red-sensitive

emulsion layer, at least one green-sensitive emulsion layer, and at least one blue-sensitive emulsion layer on its support. The order of these layers can be arbitrarily selected. A cyan forming coupler is generally incorporated in a red-sensitive emulsion layer, a magenta forming coupler in a green-sensitive layer, and a yellow forming coupler in a blue-sensitive emulsion layer, respectively, but different combinations may be used in some cases.

In the photographic light-sensitive materials according to the present invention, the photographic emulsion layers or other hydrophilic colloidal layers may contain inorganic or organic hardeners. Examples of such hardeners include, for example, chromium salts (e.g., chromium alum, chromium acetate, etc.), aldehydes (e.g., formaldehyde, glyoxal, glutaraldehyde, etc.), N-methylol compounds (e.g., dimethylolurea, methylol-dimethylhydantoin, etc.), dioxane derivatives (e.g., 2,3-dihydroxydioxane, etc.), active vinyl compounds (e.g., 1,3,5-triacyloyl-hexahydro-s-triazine, 1,3-vinylsulfonyl-2-propanol, etc.), active halogen compounds (e.g., 2,4-dichloro-6-hydroxy-s-triazine, etc.), mucohalogen acids (e.g., mucochloric acid, mucophenoxychloric acid, etc.), and the like. These hardeners can be used alone or in combinations thereof.

In the case that the hydrophilic colloidal layers of the photographic light-sensitive materials of the present invention contain dyes or ultraviolet absorbents, they may be mordanted by cationic polymers and the like.

The light-sensitive materials prepared by the present invention may contain a color fog preventing agent, such as a hydroquinone derivative, an aminophenol derivative, a gallic acid derivative, an ascorbic acid derivative, and the like.

The hydrophilic colloidal layers of the photographic materials prepared in accordance with the present invention may contain ultraviolet absorbents. Such ultraviolet absorbents include, for example, bentotriazole compounds substituted with aryl groups as described, e.g., in U.S. Pat. No. 3,533,794, 4-thioazolidone compounds as described, e.g., in U.S. Pat. Nos. 3,314,794 and 3,352,681, benzophenone compounds as described, e.g., in Japanese Patent Application (OPI) No. 2784/71, cinnamic esters as described, e.g., in U.S. Pat. Nos. 3,705,805 and 3,707,375, butadiene compounds as described, e.g., in U.S. Pat. No. 4,045,229, benzoxazole compounds as described, e.g., in U.S. Pat. No. 3,700,455, and the like. The ultraviolet absorbents described in U.S. Pat. No. 3,499,762 and Japanese Patent Application (OPI) No. 48535/79 can also be used. Ultraviolet absorbing couplers or ultraviolet absorbing polymers may also be used.

Hydrophilic colloidal layers of the light-sensitive materials prepared in accordance with the present invention may contain water-soluble dyes for various purposes, e.g., as filter dyes or for prevention of irradiation. Examples of such dyes include oxonol dyes, hemioxonol dyes, styryl dyes, merocyanine dyes, cyanine dyes and azo dyes. Of these, oxonol dyes, hemioxonol dyes and merocyanine dyes are particularly useful.

In carrying out the present invention, known discoloration inhibitors, such as hydroquinone derivatives, gallic acid derivatives, p-alkoxyphenols, p-oxyphenol derivatives, bisphenols, etc., can be used. In addition, color image stabilizing agents can be used individually or in combination of two or more thereof.

In one of the preferred embodiments according to the present invention, there is provided a silver halide pho-

tographic light-sensitive material comprising a support having formed thereon at least two emulsion layers differing in color sensitivity and at least two emulsion layers that are sensitive to the same color but different in sensitivity, at least one of these emulsion layers containing at least one compound capable of releasing a fogging agent or a development accelerator or a precursor thereof in proportion to the amount of developed silver upon development; wherein a layer containing silver halide grains which are not substantially developed by the development processing for the light-sensitive material is provided between the two emulsion layers differing in color sensitivity.

The present invention will now be illustrated in greater detail by reference to a specific example, but it is to be understood that the present invention is not limited thereto.

## EXAMPLE

In order to evaluate effectiveness of the present invention, a multilayer color light-sensitive material composed of the following layers was prepared. The resulting sample was designated as Sample 101.

In the following formulations, the amounts of emulsions applied are expressed by silver coverages.

### Sample 101

| First Layer (Antihalation Layer):                                                                               |                                             |
|-----------------------------------------------------------------------------------------------------------------|---------------------------------------------|
| A gelatin layer containing;                                                                                     | 0.18 g/m <sup>2</sup>                       |
| Black colloidal silver                                                                                          | 0.12 g/m <sup>2</sup>                       |
| Ultraviolet absorbent C-1                                                                                       | 0.17 g/m <sup>2</sup>                       |
| Second Layer (Intermediate Layer):                                                                              |                                             |
| A gelatin layer containing;                                                                                     | 0.18 g/m <sup>2</sup>                       |
| 2,5-Di-t-pentadecylhydroquinone                                                                                 | 0.11 g/m <sup>2</sup>                       |
| Coupler C-3                                                                                                     | 0.15 g/m <sup>2</sup>                       |
| Silver iodobromide emulsion<br>(silver iodide: 1 mol %; mean grain size: 0.07 μm)                               |                                             |
| Third Layer (First Red-Sensitive Emulsion Layer):                                                               |                                             |
| A gelatin layer containing;<br>Silver iodobromide emulsion<br>(silver iodide: 4 mol %; mean grain size: 0.6 μm) | 0.72 g/m <sup>2</sup>                       |
| Sensitizing Dye I                                                                                               | 7.0 × 10 <sup>-5</sup> mol<br>per mol of Ag |
| Sensitizing Dye II                                                                                              | 2.0 × 10 <sup>-5</sup> mol<br>per mol of Ag |
| Sensitizing Dye III                                                                                             | 2.8 × 10 <sup>-4</sup> mol<br>per mol of Ag |
| Sensitizing Dye IV                                                                                              | 2.0 × 10 <sup>-5</sup> mol<br>per mol of Ag |
| Coupler C-4                                                                                                     | 0.093 g/m <sup>2</sup>                      |
| Coupler C-5                                                                                                     | 0.31 g/m <sup>2</sup>                       |
| Coupler C-6                                                                                                     | 0.010 g/m <sup>2</sup>                      |
| Fourth Layer (Second Red-Sensitive Emulsion Layer):                                                             |                                             |
| A gelatin layer containing;<br>Silver iodobromide emulsion<br>(silver iodide: 6 mol %; mean grain size: 1.5 μm) | 1.6 g/m <sup>2</sup>                        |
| Sensitizing Dye I                                                                                               | 5.2 × 10 <sup>-5</sup> mol<br>per mol of Ag |
| Sensitizing Dye II                                                                                              | 1.5 × 10 <sup>-5</sup> mol<br>per mol of Ag |
| Sensitizing Dye III                                                                                             | 2.1 × 10 <sup>-4</sup> mol<br>per mol of Ag |
| Sensitizing Dye IV                                                                                              | 1.5 × 10 <sup>-5</sup> mol<br>per mol of Ag |
| Coupler C-4                                                                                                     | 0.10 g/m <sup>2</sup>                       |
| Coupler C-5                                                                                                     | 0.061 g/m <sup>2</sup>                      |
| Coupler C-6                                                                                                     | 0.005 g/m <sup>2</sup>                      |
| Coupler C-7                                                                                                     | 0.046 g/m <sup>2</sup>                      |
| Fifth Layer (Third Red-Sensitive Emulsion                                                                       |                                             |

-continued

Layer):  
Silver iodobromide emulsion  
(silver iodide: 12 mol %; mean  
grain size: 2.2  $\mu\text{m}$ )  
Sensitizing Dye I

Sensitizing Dye II

Sensitizing Dye III

Sensitizing Dye IV

Coupler C-5  
Coupler C-7

Sixth Layer (Intermediate Layer):  
A gelatin layer

Seventh Layer (First Green-Sensitive Emulsion Layer):  
A gelatin layer containing;  
Silver iodobromide emulsion  
(silver iodide: 5 mol %; mean  
grain size: 0.5  $\mu\text{m}$ )  
Sensitizing Dye V

Sensitizing Dye VI

Sensitizing Dye VII

Coupler C-8  
Coupler C-9  
Coupler C-10  
Coupler C-11

Eighth Layer (Second Green-Sensitive Emulsion Layer):  
A gelatin layer containing;  
Silver iodobromide emulsion  
(silver iodide: 6 mol %; mean  
grain size: 1.5  $\mu\text{m}$ )  
Sensitizing Dye V

Sensitizing Dye VI

Sensitizing Dye VII

Coupler C-8  
Coupler C-9  
Coupler C-10  
Coupler C-11

Ninth Layer (Third Green-Sensitive Emulsion Layer):  
A gelatin layer containing;  
Silver iodobromide emulsion  
(silver iodide: 12 mol %; mean  
grain size: 2.2  $\mu\text{m}$ )

-continued

|    |                                                                |                                           |
|----|----------------------------------------------------------------|-------------------------------------------|
| 5  | Sensitizing Dye V                                              | $3.0 \times 10^{-4}$ mol<br>per mol of Ag |
|    | Sensitizing Dye VI                                             | $2.4 \times 10^{-5}$ mol<br>per mol of Ag |
|    | Sensitizing Dye VII                                            | $9.5 \times 10^{-5}$ mol<br>per mol of Ag |
|    | Coupler C-12                                                   | 0.070 g/m <sup>2</sup>                    |
|    | Coupler C-11                                                   | 0.002 g/m <sup>2</sup>                    |
|    | Coupler C-9                                                    | 0.013 g/m <sup>2</sup>                    |
| 10 | <u>Tenth Layer (Yellow Filter Layer):</u>                      |                                           |
|    | A gelatin layer containing;                                    |                                           |
|    | Yellow colloidal silver                                        | 0.04 g/m <sup>2</sup>                     |
|    | 2,5-Di-t-pentadecylhydroquinone                                | 0.031 g/m <sup>2</sup>                    |
|    | <u>Eleventh Layer (First Blue-Sensitive Emulsion Layer):</u>   |                                           |
| 15 | A gelatin layer containing;                                    |                                           |
|    | Silver iodobromide emulsion                                    | 0.32 g/m <sup>2</sup>                     |
|    | (silver iodide: 6 mol %; mean                                  |                                           |
|    | grain size: 0.4 $\mu$ m)                                       |                                           |
|    | Coupler C-13                                                   | 0.68 g/m <sup>2</sup>                     |
|    | Coupler C-14                                                   | 0.030 g/m <sup>2</sup>                    |
| 20 | <u>Twelfth Layer (Second Blue-Sensitive Emulsion Layer):</u>   |                                           |
|    | A gelatin layer containing;                                    |                                           |
|    | Silver iodobromide emulsion                                    | 0.40 g/m <sup>2</sup>                     |
|    | (silver iodide: 10 mol %; mean                                 |                                           |
|    | grain size: 1.0 $\mu$ m)                                       |                                           |
| 25 | Coupler C-13                                                   | 0.22 g/m <sup>2</sup>                     |
|    | Sensitizing Dye VIII                                           | $2.2 \times 10^{-4}$ mol<br>per mol of Ag |
|    | <u>Thirteenth Layer (Third Blue-Sensitive Emulsion Layer):</u> |                                           |
| 30 | A gelatin layer containing;                                    |                                           |
|    | Silver iodobromide emulsion                                    | 1.00 g/m <sup>2</sup>                     |
|    | (silver iodide: 10 mol %; mean                                 |                                           |
|    | grain size: 2.3 $\mu$ m)                                       |                                           |
|    | Coupler C-13                                                   | 0.19 g/m <sup>2</sup>                     |
|    | Sensitizing Dye VIII                                           | $2.3 \times 10^{-4}$ mol<br>per mol of Ag |
| 35 | <u>Fourteenth Layer (First Protective layer):</u>              |                                           |
|    | A gelatin layer containing;                                    |                                           |
|    | Ultraviolet absorbent C-1                                      | 0.14 g/m <sup>2</sup>                     |
|    | Ultraviolet absorbent C-2                                      | 0.22 g/m <sup>2</sup>                     |
|    | <u>Fifteenth Layer (Second Protective Layer):</u>              |                                           |
| 40 | A gelatin layer containing;                                    |                                           |
|    | Polymethyl methacrylate particles                              | 0.05 g/m <sup>2</sup>                     |
|    | (diameter: 1.5 $\mu$ m)                                        |                                           |

To each of the foregoing layers were further added a gelatin hardening agent C-15 and a surface active agent 45 in addition to the above components.

Compounds used for the preparation of Sample 101 are shown below.

### Polymer having a repeating unit of the formula



-continued



C-3

C-4



C-5



C-6



C-7

Polymer having a repeating unit of the formula



C-8

-continued



-continued



C-13



C-14



C-15



I



II



III



IV

-continued



V



VI



VII



VIII

#### Samples 102 to 104

Samples 102, 103 and 104 were prepared in the same manner as described for Sample 101, except that FR-Releasing Compounds (I-1), (I-6), and (I-17), respectively, were added to the 5th layer in amounts of 0.1 g/m<sup>2</sup>, 4 mg/m<sup>2</sup>, and 5 mg/m<sup>2</sup>, respectively.

#### Samples 105 to 108

Samples 105 to 108 were prepared in the same manner as for Samples 101 to 104, respectively, except that Silver Iodobromide Emulsion A having a mean grain size of 0.08 μm and a silver iodide content of 2 mol% which was prepared as follows was added to the 6th layer of Samples 101 to 104 in an amount of 0.3 g/m<sup>2</sup> as a silver coverage.

#### Preparation of Silver Iodobromide Emulsion A:

To 1,000 ml of a 2% aqueous solution of gelatin maintained at 40°C. with stirring were simultaneously added 800 ml of a 12.5% aqueous solution of silver nitrate and 50 800 ml of an aqueous solution containing 0.24% of potassium iodide and 8.58% of potassium bromide while maintaining the pAg value of the mixture at 7.7. There was obtained a non-developable silver halide emulsion having a mean grain size of 0.08 μm and a silver iodide content of 2 mol%.

Each of Samples 101 through 108 was imagewise exposed to white light and subjected to color development as described below thereby to obtain sensitivity as shown in Table 1.

Further, Sample 101 was uniformly exposed to green light and then imagewise exposed to red light to obtain a magenta image and a cyan image as shown in Figure.

In Figure, the curve A-B represents the characteristic curve of a cyan image formed in the red-sensitive layer, and the curve a-b represents the density of a magenta image formed in the green-sensitive layer by the uniform exposure to green light. Point A indicates

the fog area of a dye image and Point B indicates an area of such an exposure amount to produce a cyan image density of 1.5. The difference between the magenta density a at Exposure A and the magenta density b at Exposure B, i.e.,  $\Delta x$ , was taken as a criterion of interlayer effect from the red-sensitive layer (R) to the green-sensitive layer (G).

Each of Samples 102 through 108 was exposed and developed in the same manner as described above. The results obtained are shown in Table 1, wherein minus values of  $\Delta x$  (a-b) indicate that the density a at Exposure A was lower than the density b at Exposure B.

The development processing employed in this example was conducted as follows as 38°C.

#### Development Processing:

|                      |       |
|----------------------|-------|
| 1. Color development | 3'15" |
| 2. Bleaching         | 6'30" |
| 3. Rinsing           | 3'15" |
| 4. Fixing            | 6'30" |
| 5. Rinsing           | 3'15" |
| 6. Stabilization     | 3'15" |

The processing solution used in each step had the following formulation:

#### Color Developing Solution:

|                                    |        |
|------------------------------------|--------|
| Sodium nitrilotriacetate           | 1.0 g  |
| Sodium sulfite                     | 4.0 g  |
| Sodium carbonate                   | 30.0 g |
| Potassium bromide                  | 1.4 g  |
| Hydroxylamine sulfate              | 2.4 g  |
| 4-(N-Ethyl-N-β-hydroxyethylamino)- | 4.5 g  |
| 2-methyl-aniline sulfate           |        |
| Water to make 1,000 ml             |        |

#### Bleaching Solution:

|                                               |         |
|-----------------------------------------------|---------|
| Ammonium bromide                              | 160.0 g |
| Aqueous ammonia (28%)                         | 25.0 ml |
| Sodium (ethylenediaminetetra-acetato) ferrate | 130 g   |
| Glacial acetic acid                           | 14 ml   |
| Water to make 1,000 ml                        |         |

## Fixing Solution:

|                            |          |
|----------------------------|----------|
| Sodium tetrapolyphosphate  | 2.0 g    |
| Sodium sulfite             | 4.0 g    |
| Ammonium thiosulfate (70%) | 175.0 ml |
| Sodium bisulfite           | 4.6 g    |
| Water to make 1,000 ml     |          |

## Stabilizing Solution:

|                                      |        |
|--------------------------------------|--------|
| Formalin (27% formaldehyde solution) | 8.0 ml |
| Water to make 1,000 ml               |        |

TABLE 1

| Sample | Fine Silver Halide Grains in 6th Layer | FR-Compound in 5th Layer | Relative Sensitivity of Cyan Image | Interlayer Effect ( $\Delta x$ ) |
|--------|----------------------------------------|--------------------------|------------------------------------|----------------------------------|
| 101    | not added                              | —                        | 100                                | 0.08                             |
| 102    | not added                              | I-1                      | 129                                | -0.07                            |
| 103    | not added                              | I-6                      | 135                                | -0.09                            |
| 104    | not added                              | I-17                     | 138                                | -0.09                            |
| 105    | added                                  | —                        | 103                                | 0.07                             |
| 106    | added                                  | I-1                      | 132                                | 0.08                             |
| 107    | added                                  | I-6                      | 135                                | 0.08                             |
| 108    | added                                  | I-17                     | 138                                | 0.07                             |

As is apparent from Table 1, although Samples 102 to 104 wherein FR compounds were merely added had increased sensitivities, they showed negative interlayer effect from the red-sensitive layer onto the green-sensitive layer, resulting in serious color mixing. To the contrary, Samples 106 to 108 prepared in accordance with the present invention not only showed high sensitivities but also underwent no substantial color mixing.

While the invention has been described in detail and with reference to specific embodiments thereof, it will be apparent to those skilled in the art that various changes and modifications can be made therein without departing from the spirit and scope thereof.

## What is claimed is:

1. A silver halide light-sensitive material comprising a support having provided thereon at least two silver halide emulsion layers differing in color sensitivity, at least one of said emulsion layers containing at least one compound capable of releasing a fogging agent, a development accelerator, or a precursor thereof in proportion to the amount of silver developed upon development processing, wherein a layer containing silver halide grains which are not substantially developed by the development processing of said light-sensitive material is provided between said two emulsion layers differing in color sensitivity.

2. A silver halide light-sensitive material as in claim 1, wherein the compound capable of releasing a fogging agent, a development accelerator, or a precursor thereof is represented by formula (1), (2), or (3):



(1)

BALL—Cp—(TIME)<sub>n</sub>—FA

(2)

RED—(TIME)<sub>n</sub>—FA

(3)

5 wherein Cp represents a coupler residue capable of coupling with an oxidation product of an aromatic primary amine developing agent; BALL represents an anti-diffusible group releasable from Cp by a coupling reaction with an oxidation product of an aromatic primary amine developing agent; RED represents a compound residue capable of undergoing oxidation-reduction with an oxidation product of an aromatic primary amine developing agent; TIME represents a timing group releasable from Cp or RED upon a coupling reaction or oxidation-reduction reaction to release FA; n represents 0 or 1; and FA represents a residue containing a group capable of fogging silver halides or accelerating development or a precursor thereof and being releasable from Cp or RED upon coupling when n is 0, or releasable from TIME when n is 1.

10 15 20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8

-continued



wherein R<sub>1</sub> represents an anti-diffusible group having from 8 to 32 total carbon atoms; R<sub>2</sub> represents a halogen atom, a lower alkyl group, a lower alkoxy group, a phenyl group or a substituted phenyl group; Z represents a non-metallic atomic group forming a substituted or unsubstituted 5-membered azole ring containing from 2 to 4 nitrogen atoms; and the asterisk (\*) indicates a position to which FA or TIME is bonded.

6. A silver halide light-sensitive material as in claim 2, wherein Cp is a cyan coupler residue represented by formula (VI), (VII), (VIII), or (IX)



wherein R<sub>1</sub> represents an anti-diffusible group having from 8 to 32 total carbon atoms; R<sub>2</sub>, which may be the same or different when R<sub>2</sub> represents two or more groups, represents one or more of a halogen atom, a lower alkyl group and a lower alkoxy group; and the asterisk (\*) indicates a position to which FA or TIME is bonded.

7. A silver halide light-sensitive material as in claim 2, wherein Cp is a colorless coupler residue represented by formula (X), (XI), or (XII)



(V) 10 wherein R<sub>1</sub> represents an anti-diffusible group having from 8 to 32 total carbon atoms; R<sub>2</sub> represents a hydrogen atom, a halogen atom, a lower alkyl group or a lower alkoxy group; and the asterisk (\*) indicates a position to which FA or TIME is bonded;



wherein R<sub>1</sub> represents an anti-diffusible group having from 8 to 32 total carbon atoms; V represents an oxygen atom, a sulfur atom, or a nitrogen atom; and the asterisk (\*) is as defined above;



wherein R<sub>1</sub> and R<sub>2</sub> each represents an alkoxy carbonyl group, an aminocarbonyl group, an acyl group, a group derived from a sulfonic acid or sulfonic acid derivative corresponding to the above-described groups, a cyano group, an ammonium group or a nitrogen containing heterocyclic group which is bonded at the N-position thereof, or R<sub>1</sub> and R<sub>2</sub> may be taken together to form a 5- or 6-membered ring; and the asterisk (\*) is as defined above.

8. A silver halide light-sensitive material as in claim 2, wherein Cp is a black forming coupler residue represented by formula (XIII), (XIV), or (XV)



wherein R<sub>1</sub> represents an alkyl group having from 3 to 20 carbon atoms, a phenyl group, or a phenyl group substituted with a hydroxyl group, an amino group, or an alkyl or alkoxy group of from 1 to 20 carbon atoms; R<sub>2</sub>, which may be the same or different, represents a hydrogen atom, a halogen atom, an alkyl or alkenyl group of from 1 to 20 carbon atoms or an aryl group of from 6 to 20 carbon atoms; R<sub>3</sub>, which may be the same or different when R<sub>3</sub> represents two or more groups, represents one or more of a halogen atom, an alkyl or alkoxy group of from 1 to 20 carbon atoms and other monovalent groups; and the asterisk (\*) indicates a position to which FA or TIME is bonded.

9. A silver halide light-sensitive material as claimed in claim 2, wherein FA is represented by formula (XII) or (XXIII)



wherein R<sub>1</sub> represents an acyl group, a carbamoyl group, an alkylsulfonyl group, an arylsulfonyl group, an alkoxy carbonyl group, an aryloxy carbonyl group, or a sulfamoyl group; R<sub>2</sub> represents a hydrogen atom, an acyl group, or an aryloxy carbonyl group; R<sub>3</sub> represents a halogen atom, an alkoxy group, an alkyl group, an alkenyl group, an aryl group, an aryloxy group, an alkylthio group, an arylthio group, a carbonamido group, or a sulfonamido group; m represents 0 or an integer of from 1 to 4; when m is 2 or more, R<sub>3</sub> may be the same or different or two or more of them may be taken together to form a condensed ring; L is a divalent linking group; n represents 0 or 1; Z<sub>1</sub> represents a monocyclic or condensed hetero ring; and Z<sub>2</sub> represents an

atomic group forming a monocyclic or condensed ring together with the adjacent nitrogen atom.

10. A silver halide light-sensitive material as in claim 1, wherein the compound capable of releasing a fogging agent, a development accelerator, or a precursor thereof is present in an amount of from  $10^{-8}$  to 0.5 mols per mol of a silver halide light-sensitive emulsion in which said compound is incorporated.
11. A silver halide light-sensitive material as in claim 10, wherein the compound capable of releasing a fogging agent, a development accelerator, or a precursor thereof is present in an amount of from  $5 \times 10^{-7}$  to  $10^{-2}$  mols per mol of the silver halide light-sensitive emulsion in which said compound is incorporated.
12. A silver halide light-sensitive material as in claim 1, wherein the silver halide grains which are not substantially developed have a silver bromide content of 60 mol% or more, a silver chloride content of 30 mol% or less, and a silver iodide content of 40 mol% or less.
13. A silver halide light-sensitive material as in claim 12, wherein the silver halide grains which are not substantially developed are silver iodobromides having a silver iodide content of from 0 to about 20 mol%.
14. A silver halide light-sensitive material as in claim 13, wherein the silver halide grains which are not substantially developed are silver iodobromides having a silver iodide content of from about 0.3 to about 5 mol%.
15. A silver halide light-sensitive material as in claim 1, wherein the silver halide grains which are not substantially developed have a mean grain size of about 0.2  $\mu\text{m}$  or less.
16. A silver halide light-sensitive material as in claim 15, wherein the silver halide grains which are not substantially developed have a mean grain size of about 0.15  $\mu\text{m}$  or less.
17. A silver halide light-sensitive material as in claim 16, wherein the silver halide grains which are not substantially developed have a mean grain size of 0.10  $\mu\text{m}$  or less.
18. A silver halide light-sensitive material as in claim 1, wherein the layer containing the silver halide grains which are not substantially developed has a silver coverage of from 0.002 to 2 g/m<sup>2</sup>.
19. A silver halide light-sensitive material as in claim 18, wherein the layer containing the silver halide grains which are not substantially developed has a silver coverage of from 0.01 to 1 g/m<sup>2</sup>.

\* \* \* \* \*